

(No Model.)

W. H. H. CHILDS.  
SHEATHING PAPER.

No. 372,894.

Patented Nov. 8, 1887.

Fig. 1.



Fig. 2.



Fig. 3.



Fig. 4.



WITNESSES:

*J. A. Garfield*  
*C. Sedgwick*

INVENTOR:

*W. H. H. Childs*  
BY *Munn & Co.*

ATTORNEYS.

# UNITED STATES PATENT OFFICE.

WILLIAM H. H. CHILDS, OF BROOKLYN, NEW YORK.

## SHEATHING-PAPER.

SPECIFICATION forming part of Letters Patent No. 372,894, dated November 8, 1887.

Application filed August 6, 1887. Serial No. 246,282. (No model.)

*To all whom it may concern:*

Be it known that I, WILLIAM H. H. CHILDS, of Brooklyn, in the county of Kings and State of New York, have invented certain new and 5 useful Improvements in Sheathing-Paper, of which the following is a full, clear, and exact description.

My invention relates to the class of compound fabric—such as sheathing or disinfectant wrapping or anti-moth paper—which is made water-proof or disinfectant or of extra strength by the interposition between two or more layers of paper or other fabric of asphalt or some other water-proof or cementing or disinfecting material. In such paper it has been found that the interposed composition has a tendency to run out from between the sheets of paper, especially under the influence of heat, if the latter is placed in a vertical position, as when a roll of such paper stands on end. If a binding or hem is used to prevent this trouble, the edge of the paper is thickened. By my invention the paper is kept of uniform thickness, less paper is required, 25 thereby effecting a saving, and the material used for waterproofing or cementing or disinfecting is effectually prevented from exuding under any conditions.

The following is the description of my invention, in which reference is made to the accompanying drawings, similar letters of reference indicating corresponding parts in all the figures.

Referring to the drawings, A A represent 35 the sheets of paper out of which the compound sheet B is constructed. Over the center or other desired portion or zone of each sheet, or of one of them, the asphalt or other desired composition is applied. This may extend to 40 within a short distance of one or each edge. To the uncovered narrow strip, along the edge or edges, paste or suitable cement is applied. If, now, the two sheets are rolled together, the entire surfaces adhere. The desired portions 45 are cemented by the asphalt or other cement, a, the rest by the paste or cement, b.

Figure 1 of the drawings represents my invention as applied to protecting or pasting both margins of the sheets of paper.

50 Fig. 2 of the drawings shows my invention as applied to treating one edge only of the sheets of paper, as in such cases where it is desirable that the principal coating should ex-

tend clear to one of the edges. In this case the cement, a, is carried from one edge nearly 55 to the other, and the remaining portion of the paper is pasted together with the paste, b. It also shows how more than two layers may be used, C representing an extra piece.

Fig. 3 of the drawings shows my invention 60 as applied to sheets of paper whose four edges receive the one paste, b, and whose center receives the cement, a.

Fig. 4 of the drawings shows sheets of paper 65 to which the paste, b, is applied in three zones, with the cement, a, interposed. This sheet may be used as it is, or may be split into narrow pieces through the dotted line x x. Intermediate lines or areas of pasting, b b, afford 70 additional security in the retaining of the cement, a a, in place when the paper is not split or slitted. The two cementing materials are so chosen that each will perform its specific functions the most effectually possible. Thus, 75 if the center is to be water-proof, the usual asphaltic composition may be applied thereto, while flour paste will secure the ends so as to prevent the asphalt from running out; or a disinfectant cement may be used for the center, and the edges may be secured by glue. 80 More than two thicknesses of paper may be employed.

I do not restrict myself to any particular paste, cement, or composition, or assortment of pastes or cementing material, and the 85 method of applying the same is no part of this invention. The respective areas of application of each cement or composition may be varied also.

Having thus fully described my invention, I 90 claim as new and desire to secure by Letters Patent—

1. As an article of manufacture, the compound paper consisting of two or more layers cemented together with two or more cementing materials, each applied within definite areas. 95

2. As an article of manufacture, the compound paper consisting of two or more layers cemented together in the center by one composition and on the edges by another, substantially as shown and described. 100

WILLIAM H. H. CHILDS.

Witnesses:

JOHN G. TAIT,  
RALPH R. MABIE.